

## [54] PROCESS FOR PRINTING AND PAD DYEING POLYAMIDE FIBROUS MATERIALS

[75] Inventors: **Gerd Pelster; Volkmar Wurtz**, both of Kelkheim/Taunus; **Erich Feess**, Lorsbach/Taunus, all of Germany[73] Assignee: **Farbwerke Hoechst Aktiengesellschaft vormals Meister Lucius & Bruning**, Frankfurt/Main, Germany

[22] Filed: June 15, 1972

[21] Appl. No.: 263,157

## Related U.S. Application Data

[63] Continuation of Ser. No. 23,473, March 27, 1970, abandoned.

## [30] Foreign Application Priority Data

Apr. 1, 1969 Germany 1916627

[52] U.S. Cl. 8/54, 8/1 E, 8/21 B, 8/163

[51] Int. Cl. D06p 1/38

[58] Field of Search 8/178, 163, 1 E, 54, 21 B

## [56]

## References Cited

## UNITED STATES PATENTS

|           |         |                       |         |
|-----------|---------|-----------------------|---------|
| 3,042,477 | 7/1962  | Hadfield et al. ....  | 8/163 X |
| 3,097,043 | 7/1963  | Mills ....            | 8/163   |
| 3,660,393 | 5/1972  | Ackermann et al. .... | 8/163 X |
| 3,663,156 | 5/1972  | Meininger et al. .... | 8/163 X |
| 3,697,500 | 10/1972 | Ackermann et al. .... | 8/163 X |

## OTHER PUBLICATIONS

H. U. Schmidlin, "Preparation and Dyeing of Synthetic Fibers," 1963, pp. 218 and 391, Publ. Chapman & Hall Ltd., London.

Primary Examiner—Thomas J. Herbert, Jr.  
Attorney, Agent, or Firm—Curtis, Morris & Safford

## [57]

## ABSTRACT

Process for preparing on textile materials consisting of polyamide fibres or of their mixtures with cellulose fibres, or containing such fibres or fibre blends, prints and pad-dyeings having extremely good fastnesses to wet processing, using reactive dyestuffs for printing and padding, and fixing these dyestuffs by steaming at a pH range of from about 6 to 11, preferably of from 7 to 8.5.

3 Claims, No Drawings

## PROCESS FOR PRINTING AND PAD DYEING POLYAMIDE FIBROUS MATERIALS

This application is a continuation application of U.S. Pat. application Ser. No. 23,473, filed Mar. 27, 1970, now abandoned.

The present invention relates to a new process for printing and pad-dyeing polyamide fibrous materials.

For printing and pad-dyeing polyamide fibrous materials there are used mainly acid dyes, complex metal dyes, disperse and pigment dyestuffs. The fastness hitherto required for goods made of polyamides are more or less attained by these dyestuff types. For improving the fastnesses to wet processing, however, special operations using suitable auxiliary agents are necessary which cause detrimental hardening of the polyamide goods, as well as an undesired extension of the process and make it highly expensive. Further, in the rinsing and washing operations, especially acid dye-stuffs tend easily to staining white spots where the polyamide goods have not been printed.

It is also known that polyamide fibrous materials can be dyed by means of reactive dyestuffs under the same fixing conditions as those for acid dyestuffs, but the resulting dyeings show only moderate fastnesses to wet processing.

Articles made from polyamide fibrous materials to be employed for bedding and table-linen, however, have to meet far higher requirements as to fastnesses. Until now, woven and knitted fabrics made from polyamide fibrous materials have generally been washed at a temperature of 40°C, at most of 60°C, whereas these articles, nowadays, should be washable at boiling temperatures and, correspondingly, the prints and dyeings should resist to frequent household washings at about 95°C in a washing machine.

Thus, the hitherto existing printing and dyeing processes for polyamide goods can no longer be applied to these polyamide articles which have to be fast to boiling, due to the insufficient fastness to washing of the cited dyestuff types. For this reason, a process producing prints and dyeings on polyamide fibres having very high fastnesses to wet processing would mean a considerable advance.

It has now been found that it is possible to obtain on textile materials consisting of polyamide fibres or of their mixtures with cellulose fibres, or containing such fibres of fibre blends, prints and pad-dyeings of high fastnesses to wet processing by using reactive dyestuffs for printing and padding, and fixing these dyestuffs by steaming at a pH range of from about 6 to 11, preferably of from 7 to 8.5.

As reactive dyestuffs, all organic dyestuffs of this category can be used in the process of the invention, i.e., such dyestuffs having at least one reactive group, a precursor for such a group or a reactive substituent, which react in known manner with the hydroxy groups of cellulose materials, thus forming a covalent bond. Suitable parent components of these organic dyestuffs are especially those of the series of anthraquinone, azo and phthalocyanine dyestuffs; both the latter may contain metal or not. Examples of reactive groups and precursors thereof are the radicals of the formulae



and



in which X represents a covalent bond or the group



R being a hydrogen atom or an optionally substituted alkyl group, Y represents a  $-SO_2-$  or  $-CO-$  group and Z 10 a hydroxy group or the radical of a mono- or polybasic acid, such as a halogen atom, above all chlorine, a sulfuric acid, thiosulfuric acid or phosphoric acid radical, or an amino group substituted by alkyl or aryl radicals, or a quaternary ammonium group. Further, those reactive groups may be used, the formulae of which are in 15 analogy to the above mentioned formulae, in which, however, the sequence of the radicals  $-X-$  and  $-Y-$  has been changed. Examples of groups of said type are the vinylsulfonyl, vinylsulfonylamino,  $\beta$ -sulfato-ethylsulfonyl,  $\beta$ -thiosulfato-ethylsulfonyl,  $\beta$ -sulfato-ethylsulfonamido and the  $\beta$ -sulfato-ethylcarbonamido 20 group.

Reactive substituents in reactive dyestuffs are those 25 which can be easily split off and then leave an electrophilic radical. Examples of such substituents are halogen atoms attached to the following ring systems: quinoxaline, triazine, pyrimidine, phthalazine and pyridazine, in particular the monochlorotriazine, dichlorotriazine, trichloro-pyrimidine, dichloro-quinoxaline 30 and the dichloro-phthalazine groups.

Finally, it is also possible to use reactive dyestuffs 35 having one or more 2,2,3,3-tetrafluoro-cyclobutane-1-acroylamino groups or a radical formed by condensation of 2-N-methylamino-5-hydroxynaphthalene-7-sulfonic acid with 2,4-dichloro-6-methoxy-1,3,5-triazine.

Examples of reactive dyestuffs of the kind cited 40 above are described in U.S. Pat. Nos. 2,670,265; 2,657,205; 3,197,456; 3,349,097; 3,324,151; 3,261,823; 3,417,074; 3,278,549; 3,360,524; 3,278,516; 3,360,509 and 3,360,505 as well as in French Pat. No. 1,448,660.

According to the process of the invention printing is 45 effected using neutral printing pastes to which a product capable of splitting off alkali is added or an alkaline salt of from weak to medium strong acids, for example sodium acetate, the sodium salt of trichloro-acetic acid, sodium carbonate, sodium bicarbonate or trisodium phosphate, or else to which small amounts of alkalis are 50 added. The same goes for the pad-steam dyeing process, in that case the polyamide material is impregnated on a foulard using a slightly thickened dye bath containing besides the dyestuff also the same above-mentioned auxiliary agents, and subsequently the textiles are steamed.

The printing thickeners or combinations of thickeners 55 employed have to meet the general requirements called for in the printing of synthetic fibres as to tintorial power, sharpness of the outlines, capability of being washed out and effect relative to the feel. The thickener should have no reducing effect, it should be neutral or adjusted to neutral.

The new process can be explained using the example 60 of vinylsulfone dyestuffs. The small quantities of alkali in the printing pastes or padding liquors are necessary for converting that dyestuff being present in the form of the sulfato-ethylsulfone compound into the reactive

vinylsulfone form, in which it forms a covalent bond while reacting with the terminal  $\text{NH}_2$  groups of the polyamide, thus imparting the prints and dyeings produced remarkably good fastnesses to wet processing not attained on polyamide material until now.

1.  $\text{F}-\text{SO}_2-\text{CH}_2-\text{CH}_2-\text{O}-\text{SO}_3\text{Na} \xrightarrow{\text{alkali}} \text{F}-\text{SO}_2-\text{CH}=\text{CH}_2$
2.  $\text{F}-\text{SO}_2-\text{CH}=\text{CH}_2 + \text{H}_2\text{N-PA} \longrightarrow \text{F}-\text{SO}_2-\text{CH}_2-\text{NH-PA}$

PA = polyamide material

An excess of alkali in the pastes or liquors results in an insufficient fixation of the dyestuff. A decrease in the pH value below 6 has the same effect simultaneously combined with far poorer fastnesses to wet processing, for in this lower pH range no reaction between the dyestuff and the fibre occurs.

In the process of the invention such dyestuffs are advantageously used of which the strength of their salt-like bond to the polyamide material being relatively weak, so that the portion of not covalent fixed dyestuff is easily removable by washing out. Dyestuffs of this kind are those having at least one, preferably two and more, water-solubilizing groups, such as carboxylic acid and/or sulfonic acid groups.

In some cases, especially if complex metal dyestuffs are applied or dyestuffs containing a number of water-solubilizing groups which is too small in comparison to their molecular sizes, the dyestuff portion not being linked by a covalent bond, i.e., in a salt-like manner only, is absorbed onto the fibre more powerfully, thus faster to washing. This portion of the dye, however, remains on the fibre occasionally in the washing operation under mild conditions disclosed before so that, thereupon, the results of a later, more severe washing test would be correspondingly poorer.

But in this event, an after-treatment of the prints or pad-dyeings obtained by using the foregoing-mentioned dye-stuffs with an aqueous weakly alkaline solution, preferably with dilute ammonia, will quantitatively remove the excess dyestuff likewise. The remaining reactively bound dyestuff then shows very good fastnesses to wet processing.

According to the printing and pad-dyeing process of the invention, the cellulose fibre portion of the fibre mixtures with polyamide fibres may be of native or regenerated origin.

Fixing of the prints and pad-dyeings is carried out by steaming at temperatures ranging between 98° and 130° C. In order to get a uniform and optimum dyestuff fixation, steaming periods are necessary which are generally between 10 and 30 minutes. The color yield is improved by steaming under elevated pressures (up to 1.5 atmospheres gauge). The polyamide material can be treated either in discontinuously operating steamers, for example in a star steamer, or in continuously operating steamers, such as Krostewitz, Mather-Platt or suspension-loop steamers etc. But continuous steamers cannot be operated under atmospheric excess pressure, and therefore the color yield on polyamide fibres, obtained by using this equipment, is correspondingly lower.

This disadvantage can be eliminated according to the process of the invention by a pre-treatment of the polyamide material, before its printing or dyeing, with water or steam at elevated temperatures of up to about 130° C and under atmospheric excess pressure (of up

to 1.5 atmospheres gauge), which treatment results in a certain swelling of the fibre, especially in a partial splitting of the  $-\text{NH-CH}_2-\text{CO-}$  chains of the polyamide with the simultaneous formation of new terminal amino groups suitable for binding the dyestuffs. Consequently, in the case of polyamide material pre-treated in the above manner it is possible, after the printing or dyeing operation, to steam the goods continuously at a temperature of about 102° C without an excess pressure and to obtain a substantially higher color yield than on goods which are not pre-treated. A discontinuous pressure steam treatment of the printed or padded polyamide goods thus is unnecessary, because it does not lead to further substantial increase in color yield.

According to the simplest way, the pre-treatment is carried out in one operation along with the usual pre-washing or hydrofixing of the goods, at a pressure of from 0.5 to 1.5 atmospheres gauge, and at a temperature between 108° and 130° C in a neutral or, preferably, weakly alkaline medium; a greater number of terminal amino groups being formed in this weakly alkaline medium. The polyamide material may also be pre-treated by steaming in a star steamer at a pressure of from 0.5 to 1.5 atmospheres gauge without or, preferably, after having been impregnated using small amounts of alkali or of products capable of splitting off alkali (for example a solution of 10 g of sodium acetate per litre of water).

At the final rinsing and washing process after the printing and steaming of the goods, the technical progress of the process of the invention resides in the fact that washing and rinsing can be carried out in a neutral or weakly alkaline medium, at which dyestuff that is fixed merely like an acid dyestuff not only has no dyeing effect, but is completely stripped from the textile material. Under the same conditions normal acid dyestuffs would show very heavy bleeding effects. Just so, the separate process for improving the fastness to wet processing, otherwise usual up to now, is no longer necessary.

The following Examples illustrate the invention; parts and percentages being by weight unless otherwise stated.

#### EXAMPLE 1

50 g of the dyestuff of the formula



65

are dissolved in 250 g of boiling water. The solution is stirred into 500 g of an aqueous thickener of 9 percent strength comprising an ether of locust bean flour. Sub-

sequently, 15 g of the sodium salt of trichloro-acetic acid, dissolved in water at a ratio of 1:1, and finally, 185 g of cold water are added to the paste.

A fabric made of polyamide-6 fibres is printed by means of the above printing paste, then dried and subsequently steamed for 30 minutes in a star steamer at about 112° C and at 0.5 atmosphere gauge. Finally, the goods are rinsed and washed with cold and warm water and then soaped in an aqueous bath at about 80° C, with addition of an anion-active detergent.

A yellow print having good fastness to wet processing is obtained.

#### EXAMPLE 2

50 g of the dyestuff of the formula



are dissolved in 250 g of boiling water and stirred into 500 g of an aqueous thickener of 9 percent strength comprising an ether of locust bean flour. Subsequently, 15 g of sodium acetate, dissolved in water at a ratio of 1:1, and 185 g of cold water are added to the paste.

A knitted fabric made of polyamide-6.6 fibres is printed by means of the above printing paste and subsequently dried. The fabric is then steamed for 20 minutes in a star steamer at 1.5 atmospheres gauge and about 126°-128° C.

Finally, the goods are rinsed in cold and warm water and soaped in an aqueous bath at about 80° C, while adding a detergent. A red print having good fastnesses is obtained.

#### EXAMPLE 3

50 g of the dyestuff of the formula



are dissolved in 250 g of boiling water. The solution is stirred into 500 g of an aqueous thickener of 9 percent strength comprising an ether of locust bean flour. Subsequently, 5 g of disodium phosphate and 195 g of cold water are added to the paste.

A fabric made of polyamide fibres is printed by means of the above paste and then dried. Subsequently, the goods are steamed continuously in a suspension loop steamer for 30 minutes at about 102°-104° C. Rinsing of the fabric in cold and hot water is effected with the addition of 1 to 1.5 cc of a 25 percent ammonia, per litre of liquor. Then the goods are soaped in an aqueous bath while adding the same amount of ammonia and together with a detergent, at temperatures between 60° and 80° C.

A brilliant, deep blue print having good fastness properties is obtained.

#### EXAMPLE 4

100 g of the dyestuff of the formula



are dissolved in 300 g of boiling water. The solution is stirred into 500 g of a thickener, consisting of a mixture of equal parts of a 25 percent aqueous thickening of crystal gum and of a 10 percent aqueous thickening of a vegetable flour derivative. Subsequently, 20 g of sodium acetate, dissolved in water at a ratio of 1:1, 10 g of the sodium salt of m-nitrobenzenesulfonic acid as oxydation agent, as well as 70 g of cold water are added to the paste.

A fabric consisting of a mixture of 60 percent polyamide fibres and 40 percent of cellulose fibres is printed by means of the above printing paste and then dried. Steaming of the goods is effected for 20 minutes in a star steamer at 0.5 atmospheres gauge and about 112° C.

Finally, the goods are rinsed in cold and warm water and soaped in an aqueous bath at about 80° C, with addition of a non-ionic detergent.

A black print having good fastness properties is obtained.

#### EXAMPLE 5

50 g of the dyestuff of the formula



are dissolved in 250 g of boiling water. Into this solution 150 g of a 10 percent aqueous solution of sodium alginate are added. Subsequently, 10 g of  $\text{Cl}_3\text{C}-\text{COONa}$ , dissolved in water at a ratio of 1:1 and 540 g of cold water are added.

A fabric made of polyamide fibres is padded by means of the above padding bath and then dried. Steaming of the goods is effected for 20 minutes in a star steamer at about 112° C and 0.5 atmospheres gauge. Subsequently, the goods are rinsed with cold and warm water and soaped in an aqueous bath while a detergent is added.

An orange dyeing having good fastness properties is obtained.

#### EXAMPLE 6

50 g of the dyestuff of the formula



are mixed with 50 g of urea and dissolved in 250 g of boiling water. The solution is stirred into 500 g of an aqueous thickener of 10 percent strength comprising an ether of locust bean flour. Thereupon 15 g of  $\text{CCl}_3\text{COONa}$ , dissolved in water at a ratio of 1:1, and finally 135 g of cold water are added to the paste.

A knitted fabric made of polyamide fibres, pre-treated in a high temperature equipment at an atmospheric excess pressure of 1.5 atmospheres gauge and at 128° C, at a pH of 8 using an aqueous medium with addition of  $\text{CH}_3\text{COONa}$ , is printed by means of the above printing paste and then dried. Subsequently, the goods are steamed for 20 to 30 minutes in a continuous steamer at about 102° C without the application of atmospheric excess pressure. Finally, the material is rinsed with cold and warm water and soaped in an aqueous bath at about 80° C while a detergent is added.

A scarlet red print having good fastness properties is obtained.

#### EXAMPLE 7

50 g of the dyestuff of the formula



are mixed with 50 g of urea and dissolved in 250 g of boiling water. The solution is stirred into 500 g of an aqueous thickener of 10 percent strength comprising an ether of locust bean flour. Further, there are added to the paste 10 g of  $\text{CH}_3\text{COONa}$  and 140 g of cold water.

A fabric made of polyamide fibres, pre-treated with steam in a star steamer at an excess pressure of 1.5 atmospheres gauge and a temperature of 128° C, is printed by means of the above printing paste and then dried. Then the goods are steamed and finished according to Example 6.

An orange print having good fastness properties is obtained.

#### EXAMPLE 8

50 g of the dyestuff of the formula



are dissolved in 250 g of boiling water. This solution is stirred into 500 g of an aqueous thickener of 10 percent strength comprising an ether of locust bean flour. Thereupon, 5 g of  $\text{Na}_2\text{H PO}_4$  and 195 g of cold water are added to the paste.

A fabric consisting of a mixture of 80 percent of polyamide fibres and 20 percent of cotton fibres, impregnated with a 1 percent aqueous solution of sodium acetate and pre-steamed in a star steamer at 1.5 atmospheres gauge and 128° C, is printed by means of the above printing paste and then dried. Steaming and finishing of the goods are effected as in Example 6.

A red print of good color intensity and good fastness properties is obtained.

#### EXAMPLE 9

50 g of the dyestuff of the formula



are dissolved in 250 g of boiling water and stirred into 500 g of an aqueous thickener of 10 percent strength comprising a vegetable flour. Subsequently, 15 g of  $\text{CH}_3\text{COONa}$  and 185 g of cold water are added to the paste.

A fabric made of polyamide fibres, pre-steamed in a high temperature equipment at 0.5 to 1.5 atmospheres gauge and 108° to 130° C, is printed by means of the above printing paste and then dried. Subsequently, the fabric is steamed and finished according to Example 6.

A deep red print having good fastness properties is obtained.

#### EXAMPLE 10

50 g of the dyestuff of the formula



are mixed with 50 g of urea, dissolved in 250 g of boiling water and then stirred into 500 g of an aqueous thickener of 10 percent strength comprising a vegetable flour. Finally, 10 g of  $\text{CH}_3\text{COONa}$  and 140 g of cold water are added to the paste.

A fabric made of polyamide fibres, pre-treated according to Example 6, is printed by means of the above printing paste and then dried. Subsequently, the material is steamed and washed as in Example 6.

A red print having good fastness properties is obtained.

#### EXAMPLE 11

50 g of the dyestuff of the formula



are mixed with 50 g of urea and dissolved in 250 g of boiling water. The solution is stirred into 500 g of an aqueous thickener of 10 percent strength comprising an ether of locust bean flour, then 15 g of  $\text{CCl}_3\text{COONa}$ , dissolved in water at a ratio of 1:1, as well as 135 g of cold water are added to the paste.

A fabric made of polyamide fibres, pre-treated as in Example 6, is printed by means of the above printing

paste and then dried. Subsequently, the material is steamed and finished as in Example 6.

A blue print having good fastness properties is obtained.

#### EXAMPLE 12

50 g of the dyestuff of the formula



are dissolved in 250 g of boiling water and stirred into 500 g of an aqueous thickener of 10 percent strength comprising an ether of a vegetable flour. Subsequently, 10 g of  $\text{CH}_3\text{COONa}$  and 190 g of cold water are added to the paste.

This printing paste is applied as in Example 6. A yellow print having good fastnesses is obtained.

#### EXAMPLE 13

50 g of the dyestuff of the formula



are mixed with 50 g of urea and dissolved in 250 g of boiling water. The solution is stirred into 500 g of an aqueous thickener of 10 percent strength comprising an ether of a vegetable flour. Finally, 10 g of  $\text{CH}_3\text{COOHa}$  and 140 g of cold water are added to this paste.

A knitted article made from polyamide fibres, pre-treated as in Example 6, is printed by means of the above printing paste and then dried. Thereupon, the goods are steamed continuously for 30 minutes at about 103° C without the application of atmospheric excess pressure. Subsequently, they are rinsed in cold and warm water and soaped in an aqueous bath at about 80° C while a detergent is added.

A red print having good fastness properties is obtained.

We claim:

1. A process for preparing a print or pad-dyeing having good fastness to wet processing on a textile material containing polyamide fibers which comprises: applying to said material a printing paste or a padding liquor containing a water-soluble reactive dyestuff, containing a compound capable of splitting off alkali or a sodium or potassium salt of a weak to medium strong acid and having a pH of from about neutral to about 8.5; and fixing said reactive dyestuff on the fibers by steaming.

2. A process according to claim 1 wherein said fixing is by steam at a temperature of about 98° C. to about 130° C. at a pressure of about atmospheric to about 1.5 atmospheres gauge.

3. A process according to claim 1 which further comprises washing said textile material subsequent to said fixing in a weakly alkaline aqueous bath.

\* \* \* \* \*